# NEW EUROPEAN PATENT SPECIFICATION

(11) **EP 1 122 084 B2**
(45) Date of publication and mention of the opposition decision: **02.07.2008**
(45) Mention of the grant of the patent: 15.12.2004
(21) Application number: 01300765.3
(22) Date of filing: 29.01.2001
(51) Int. Cl.: B41M 5/00

(54) **Ink-jet recording material suitable for pigment ink**
Für eine pigmenthaltige Tinte geeignetes Tintenstrahlaufzeichnungsmaterial
Matériau d' enregistrement à jet d' encre adapté pour encre à pigment

(30) Priority: 31.01.2000 JP 2000023431; 17.01.2001 JP 2001008679
(43) Date of publication of application: 08.08.2001
(73) Proprietor: NIPPON PAPER INDUSTRIES CO., LTD., Kita-ku, Tokyo (JP)
(72) Inventor: Kondo, Noboru, c/o Res. Lab. of Product Dev., 1-chome, Shinjuku-ku, Tokyo (JP); Otani, Teiichi, c/o Res. Lab. of Product Dev., 1-chome, Shinjuku-ku, Tokyo (JP); Ono, Atsushi, c/o Res. Lab. of Product Dev., 1-chome, Shinjuku-ku, Tokyo (JP)
(74) Representative: Wilson Gunn

(56) References cited:
- EP-A- 0 803 374
- EP-A- 0 875 394
- EP-A- 0 887 199
- EP-A- 0 943 450
- EP-A- 0 958 933
- EP-B- 0 705 172
- DE-A- 19 534 327
- JP-A- 59 096 988
- JP-A- 62 085 981
- US-A- 4 446 174

## Description

### FIELD OF THE INVENTION

The present invention relates to a recording material for ink-jet process. In particular, the invention is concerned with an ink-jet recording material that can ensure good ink absorption and excellent color reproduction even when images are recorded thereon by a full color ink-jet process using pigment ink.

### BACKGROUND OF THE INVENTION

The ink-jet recording method is a recording method of forming ink images on a recording material by directing jets of ink drops at the recording material by the use of various techniques. This recording method enables high-speed and full-color printing to be easily achieved with a low noise level. In recent years, therefore, the utilization of ink-jet recording methods has been spreading at a rapid rate. According to such a method, fine drops of ink are jetted from nozzles at a high speed so as to direct toward a recording material. And a large quantity of solvent is contained in the ink used. As a result, recording materials for ink-jet recording are required to absorb ink promptly.

The recent years have also seen rapid proliferation of personal computers and digital cameras. Under these circumstances, image qualities on a level similar to those attained by silver salt photography have come to be required for images printed from digital image information. In other words, it has become necessary that, in printing images of digital information origin, recording materials can ensure high-density colors, high resolution and excellent color reproduction in the prints obtained.

In full color recording, ink-jet printers using the so-called dye ink rank as the dominant printers. This is because the dye ink generally comprises at least three kinds of ink prepared by dissolving dyes of different colors in separate portions of a solvent respectively and the dyes comprised therein as coloring ingredients are superior in point of color formation. On the other hand, ink-jet printers using the so-called pigment ink are employed for specific purposes alone under the current circumstances. The pigment ink used therein comprises at least three kinds of ink, wherein pigments of at least three different colors are dispersed as their respective main coloring ingredients and water is used as their respective main dispersion media. The purposes for using them center chiefly on the printing of rough images, e.g., wide-format images including poster. This is because the images printed in pigment ink are inferior in color reproduction though they have excellent light resistance and water resistance.

In general, ink-jet recording materials designed placing importance on ink absorption are provided with an ink-receiving layer having minute pores for promoting penetration of ink. When pigment ink is used in recording on a recording material designed for dye-ink use, it sometimes occurs that pigment particles stop up the foregoing minute pores. In this case, ink absorption becomes bad, and pigments as coloring ingredients are confined within a very thin surface region of the ink-receiving layer. As a result, the rubbing resistance of recorded images deteriorates.

On the other hand, when the pores present in an ink-receiving layer are greater in size than pigment particles, the pigments as coloring ingredients penetrate too deeply in the ink-receiving layer. As a result, the images recorded are inferior in color density and color reproduction. As matters stand, therefore, no recording materials capable of delivering both excellent color reproduction and high ink absorption when pigment ink is used are known yet.

As an answer to such a problem, Japanese Tokkai Hei 10-119417 (the term "Tokkai" as used herein means an "unexamined published patent application") proposes providing a layer which can swell in ink by containing a water-soluble resin on an ink penetration layer containing an inorganic filler. However, such an ink absorption layer is slow in ink drying speed, and so it has an image formation problem.

Further, Japanese Tokkai Hei 11-254818 discloses the recording sheet provided with an ink-receiving layer containing silica grains. However, such a sheet has insufficient color reproduction.

EP-A-943450 discloses an ink-jet recording sheet having on a support an ink receiving layer comprising pigment, binder and magnesium chloride.

JP-A-6285981 and EP-A-958933 disclose ink-jet recording sheets.

### SUMMARY OF THE INVENTION

Therefore, an object of the invention is to provide a recording material suitable for an ink-jet process using pigment ink, which can well absorb pigment ink, cause no bleed and ensure high color density and excellent color reproduction when images are printed thereon with a printer using pigment ink.

The aforementioned object is attained with an ink-jet recording material suitable for pigment ink, which has on a support at least two ink-receiving layers comprising pigment and binder: with the uppermost layer of the ink-receiving layers further containing at least one water-soluble metal salt which is selected from the group consisting of aluminium salts, magnesium salts, sodium salts, potassium salts and zinc salts and presents a pH around 7 or below when dissolved in water (namely, which is neutral or acidic), wherein the water-soluble metal salt is contained in an amount of 0.5 to 10 parts by weight per 100 parts by weight of pigment in the uppermost ink-receiving layer, and the constituent anion of the metal salt is a sulphate or thiosulfate ion.

### DETAILED DESCRIPTION OF THE INVENTION

The term "pigment ink" as used in the invention is intended to include not only unmixed pigment ink but also ink mixtures of at least 50 weight % of pigment ink and less than 50 weight % of dye ink, or the so-called dye pigment ink.

The coloring component of pigment ink may be any of organic and inorganic pigments, and it is present in a state of being dispersed in an ink solvent.

Aluminum salts, magnesium salts, sodium salts, potassium salts and zinc salts used in the invention are required to be salts soluble in water at room temperature.

In particular, sulfate ion is used to advantage because it can produce great effect in only a small amount. Examples of a water-soluble salt suitable for the invention include aluminum sulfate, magnesium sulfate, sodium thiosulfate and potassium thiosulfate.

From the viewpoints of color reproduction of recorded images and production cost of recording materials, magnesium sulfate is most suitable as a water-soluble salt used in the invention. Additionally, two or more of the water-soluble metal salts recited above may be used as a mixture in the present recording material.

Of the ink-receiving layers that are provided on a support to constitute the present recording material, the layer in which the present water-soluble metal salt or salts are incorporated is the outermost ink-receiving layer. The suitable amount of water-soluble salt(s) incorporated is from 0.5 to 10 parts by weight, preferably from 1 to 8 parts by weight, per 100 parts by weight of pigment in the outermost ink-receiving layer. Since the water-soluble salts recited above have an effect of fixing pigment ink to an ink-receiving layer, they enable the ink images to have high densities and satisfactorily reproduced colors. When the amount of water-soluble salt(s) incorporated is smaller than 0.5 parts by weight, the water-soluble salt(s) cannot satisfactorily produce the effect thereof. On the other hand, when the water-soluble metal salt or salts are incorporated in an amount greater than 10 parts by weight, they may have bad influences upon ink absorption and other characteristics.

The present recording material has no particular restrictions on a support used therein. For instance, the support used may be transparent or opaque. More specifically, depending on the desired purpose thereof, the support can be selected from among various plastic films, including films of cellophane, polyethylene, polypropylene, soft polyvinyl chloride, hard polyvinyl chloride and polyester, or a wide variety of paper including wood-free paper, base paper for photographic paper, drawing paper, painting paper, coated paper, art paper, cast-coated paper, craft paper, laminated paper, impregnated paper and synthetic paper.

When the support used is a film having substantially no absorbing capacity, it is required to take a certain measure, such as a measure of increasing the coverage of an ink-receiving layer or using a pigment having higher absorbing capacity in an image-receiving layer. In the case of employing a printer having higher resolution in particular, the larger amount of ink is struck into per-unit area of a recording sheet. So, it is required for the recording sheet in its entirety to have the higher ink absorptive capacity.

The total coverage of ink-receiving layers may be determined so as to balance against the ink absorptive capacity of a support used. Specifically, the desired color reproduction can be achieved when the ink-receiving layers have their total coverage within the range of 5 to 40 g/m². When the ink-receiving layers have a total coverage lower than 5 g/m², there sometimes occurs a difference in ink absorption speed at the interface between a support and the lowest ink receiving layer even when a material used as the support has a very good ink absorptive capacity. As a result, bleeding is caused noticeably in image areas, particularly in image areas of mixed colors. On the other hand, when the ink-receiving layers have their total coverage higher than 40 g/m², the ink applied thereto can penetrate deeply into them to result in lowering of coloring performance. In addition, it sometimes happens that the ink-receiving layer is powdered on the surface by slight external forces and comes off in powder or exfoliates when ink-image areas are rubbed. In other words, the ink-receiving layer surface tends to have a strength problem.

It is advantageous to provide an ink-receiving layer in a multi-layer structure from the viewpoint of improvement in ink absorptive capacity. In the case of the ink-receiving layer having a multi-layer structure, the outermost ink-receiving layer containing a water-soluble metal salt is preferably provided at a coverage of at least 3 g/m² for serving a function as a pigment ink-fixing layer.

Suitable examples of pigments usable in the present ink-receiving layers include precipitated calcium carbonate, ground calcium carbonate, kaolin, clay, talc, titanium dioxide, zinc oxide, zinc carbonate, satin white, magnesium carbonate, magnesium silicate, calcium sulfate, calcium silicate, aluminum silicate, aluminum hydroxide, alumina sol, colloidal alumina, alumina such as psuedo-boehmite or hydrated alumina, zeolite, silica, and plastic pigments. Of these pigments, synthetic silica is preferably used in the invention. For further attaining the desired ink absorptive capacity as the coverage of ink-receiving layers is controlled to the range in which no layers come off in powder, it is favorable to use a pigment having an oil absorption of 100 to 300 cc/100 g.

Examples of a binder usable in the present ink-receiving layers include various kinds of starch, such as oxidized starch, esterified starch, enzyme-denatured starch and cationic starch, proteins such as casein and soybean protein, cellulose derivatives such as carboxymethyl cellulose and hydroxyethyl cellulose, water-soluble high molecular compounds such as polyvinyl alcohols different in saponification degree and derivatives thereof, and water-dispersible high molecular compounds such as acrylic resin emulsions, vinyl acetate resin emulsions, vinylidene chloride resin emulsions, styrenebutadiene latex, acrylonitrile-butadiene latex and a polyester dispersion. Of course, these examples should not be construed as limiting the binders usable in the present ink-receiving layers, but any materials can be employed as the binder as far as they have strong adhesion to the support and form films after drying. Such binders may be used alone or as a mixture of two or more thereof.

The suitable amount of binder added, though varies to some extent depending on the kind of pigment used together, is in the range of 5 to 60 parts by weight, preferably 10 to 50 parts by weight, per 100 parts by weight of pigment. This is because the ink-receiving layer has a surface strength problem when it contains a binder in an amount smaller than 5 parts by weight, while when the amount of binder added is larger than 60 parts by weight the ink absorptive capacity of the resulting layer becomes insufficient.

In addition, various additives, such as a thickener, an antifoaming agent, a defoaming agent, a pigment-dispersing agent, a release agent, a blowing agent, a pH controlling agent, a surface-sizing agent, a coloring dye, a coloring pigment, a fluorescent dye, a UV absorbent, an antioxidant, a light stabilizer, an antiseptic, a waterproof agent, a dye fixing agent, a surfactant and a wet paper strength increasing agent, can be added in appropriate amounts to the ink-receiving layers so far as the addition thereof does not impair the effects of the invention.

The ink-receiving layers can be provided on a support by using a known coating apparatus, such as a blade coater, a roll coater, an air knife coater, a bar coater, a curtain coater, a gravure coater, a gate roll coater, a short dwell coater and a size press, under an on-machine or off-machine condition. In addition, a transfer method can also be adopted wherein ink-receiving layers are coated on a support and a film respectively and then brought into face-to-face contact to be bonded together.

Further, various kinds of calendering apparatus, such as a machine calender, a super calender and a soft calender, can be used alone or in combination for finishing the layer surface.

Now, specific constitutions of recording materials according to the invention are illustrated by reference to the following examples and characteristics of the present recording materials are explained by putting them in contrast with those of comparative recording materials. However, it should be understood that these examples are not to be construed as limiting the scope of the invention in any way. Unless otherwise noted, all "parts" and all "%" are by weight in the following examples and comparative examples.

Performance evaluations of recording materials prepared for pigment ink jet recording in the following Examples and Comparative Examples are made using the following methods.

### Pigment Ink Jet Recording Test

The established solid and image patterns are recorded on each of recording material samples with an ink-jet printer for pigment-ink use, HP DesignJet 2500 CP (made by HEWLETT PACKARD CO.) in which the pigment ink for exclusive use thereof is installed, and evaluated by the following criteria.

### (1) Color Reproduction:

The black, cyan, magenta and yellow solid patterns are examined for their respective densities by means of a Macbeth densitometer, RD915 (made by Macbeth Co.) . Color reproduction of each sample is graded by the sum total of measured values of those color densities.
ⓞ: 6.0 < sum total of measured values
○: 5.0 ≤ sum total of measured values ≤ 6.0
Δ: 4.0 ≤ sum total of measured values < 5.0
X: sum total of measured values < 4.0

### (2) Ink Absorption:

A pattern constituted of areas solidly colored in red (mixture of magenta ink and yellow ink) and those solidly colored in green (mixture of cyan ink and yellow ink) which are arranged so as to border on one another is printed on each sample, and the extent of bleed on the borders is evaluated by visual observation according to the following criteria. Additionally, the bleed on the border between red and green areas has a black color, so the observation thereof enables clear-cut evaluation.
ⓞ: Absolutely no bleed is observed on the borders
○: Practically no bleed is observed on the borders
Δ: A little bleed is observed on the borders
×: Considerable bleed is observed on the borders

### EXAMPLE 1

Ninety parts of hardwood kraft pulp (L-BKP) and 10 parts of softwood kraft pulp (N-BKP) were mixed, and beaten till the pulp mixture had a freeness of 350 ml in terms of csf (Canadian standard freeness). The resulting pulp was admixed with 4 parts of cationic starch, 0.3 parts of anionic polyacrylamide and 0.5 parts of an alkylketene dimer emulsion, and made into paper in a conventional way using a Fourdrinier paper machine, followed by predrying. Thereafter, a solution containing 5 % of phosphorylated starch and 0.5 % of polyvinyl alcohol was coated on the paper so as to have a coverage of 4 g/m² on a solids basis by means of a size press, and subjected to machine caledering treatment. The base paper thus made had a basis weight of 100 g/m².

On this base paper, the following coating Composition (1) was coated at a coverage of 10 g/m² on a solids basis by means of a bar blade coater, and treated using a calendering apparatus under a linear pressure of 80 kg/cm. Further thereon, the following coating Compositions (2) was coated with a bar blade coater so as to have a coverage of 5 g/m² on a solids basis, dried till the water content therein was reduced to 5 %, and then treated using a calendering apparatus under a linear pressure of 100 kg/cm, thereby forming a ink-jet recording material having a basis weight of 115 g/m². Additionally, the following amount of every ingredient except water mixed in the coating Compositions (1) and (2) is shown on a solid basis

### Coating Composition (1):

| | |
|---|---|
| Synthetic silica (X-12, trade name, a product of Tokuyama Corp.) | 100 parts |
| Polyvinyl alcohol (PVA 117, trade name, a product of Kuraray Co., Ltd.) | 35 parts |
| Dye fixing agent (PAS-H-10L, trade name, a product of Nitto Boseki Co., Ltd.) | 5 parts |
| Water | 640 parts |

### Coating Composition (2):

| | |
|---|---|
| Synthetic silica (X-12, trade name, a product of Tokuyama Corp.) | 100 parts |
| Polyvinyl alcohol (PVA 117, trade name, a product of Kuraray Co., Ltd.) | 35 parts |
| Water-soluble magnesium salt (magnesium sulfate heptahydrate (on an anhydrous basis)) | 8 parts |
| Dye fixing agent (PAS-H-10L, trade name, a product of Nitto Boseki Co., Ltd.) | 5 parts |
| Water | 640 parts |

### EXAMPLE 2

A recording material was prepared in the same manner as in Example 1, except that the amount of magnesium sulfate heptahydrate mixed in the coating Composition (2) was reduced to 4 parts on an anhydrous basis.

### EXAMPLE 3

A recording material was prepared in the same manner as in Example 1, except that the amount of magnesium sulfate heptahydrate mixed in the coating Composition (2) was reduced to 2 parts on an anhydrous basis.

### EXAMPLE 4

A recording material was prepared in the same manner as in Example 1, except that the amount of magnesium sulfate heptahydrate mixed in the coating Composition (2) was reduced to 0.5 parts on an anhydrous basis.

### EXAMPLE 5

A recording material was prepared in the same manner as in Example 1, except that aluminum sulfate octadecahydrate in an amount of 4 parts on an anhydrous basis was mixed in the coating Composition (2) in place of the magnesium sulfate heptahydrate.

### EXAMPLE 6

A recording material was prepared in the same manner as in Example 1, except that sodium thiosulfate pentahydrate in an amount of 4 parts on an anhydrous basis was mixed in the coating Composition (2) in place of the magnesium sulfate heptahydrate.

### EXAMPLE 7

A recording material was prepared in the same manner as in Example 1, except that sodium sulfate decahydrate in an amount of 4 parts on an anhydrous basis was mixed in the coating Composition (2) in place of the magnesium sulfate heptahydrate.

### EXAMPLE 8

A recording material was prepared in the same manner as in Example 1, except that potassium thiosulfate trihydrate in an amount of 4 parts on an anhydrous basis was mixed in the coating Composition (2) in place of the magnesium sulfate heptahydrate.

### EXAMPLE 9

A recording material was prepared in the same manner as in Example 1, except that 4 parts of potassium sulfate was mixed in the coating Composition (2) in place of the magnesium sulfate heptahydrate.

### EXAMPLE 10

A recording material was prepared in the same manner as in Example 1, except that zinc sulfate heptahydrate in an amount of 4 parts on an anhydrous basis was mixed in the coating Composition (2) in place of the magnesium sulfate heptahydrate.

### EXAMPLE 11

A recording material was prepared in the same manner as in Example 1, except that magnesium thiosulfate hexahydrate in an amount of 4 parts on an anhydrous basis was mixed in the coating Composition (2) in place of the magnesium sulfate heptahydrate.

### EXAMPLE 12

A recording material was prepared in the same manner as in Example 2, except that the coverage of the coating Composition (1) was decreased to 0.5 g/m² on a solids basis and the coverage of the coating Composition (2) was decreased to 3 g/m² on a solids basis.

### EXAMPLE 13

A recording material was prepared in the same manner as in Example 2, except that the coverage of the coating Composition (1) was increased to 30 g/m² on a solids basis.

### EXAMPLE 14

A recording material was prepared in the same manner as in Example 2, except that the base paper used as support was replaced by a double-side thermoplastic resin-laminated paper (Oper®, trade name, a product of Nippon Paper Industries Co., Ltd.) and the coverage of the coating Composition (1) was increased to 30 g/m² on a solids basis.

### COMPARATIVE EXAMPLE 1

A recording material was prepared in the same manner as in Example 1, except that magnesium carbonate trihydrate in an amount of 4 parts on an anhydrous basis was mixed in the coating Composition (2) in place of the magnesium sulfate heptahydrate.

### COMPARATIVE EXAMPLE 2

A recording material was prepared in the same manner as in Example 1, except that the amount of magnesium sulfate heptahydrate mixed in the coating Composition (2) was reduced to zero.

### COMPARATIVE EXAMPLE 3

A recording material was prepared in the same manner as in Example 2, except that the coating Composition (2) was used for the first layer on the base paper and the coating Composition (1) was used for the second layer on the base paper.

### COMPARATIVE EXAMPLE 4

A recording material was prepared in the same manner as in Example 1, except that ferrous sulfate heptahydrate in an amount of 4 parts on an anhydrous basis was mixed in the coating Composition (2) in place of the magnesium sulfate heptahydrate.

Results of evaluating suitability of the recording materials prepared in Examples 1 to 14 and Comparative Examples 1 to 4 respectively for pigment ink jet printing are shown in Tables 1 and 2. Additionally, the recording materials can be used without any particular problems when graded ⓞ to Δ for their performances as shown in the Tables.

**Table 1**

| Example No. | First Layer | Second Layer (uppermost layer) | | | Evaluation Results | | Note |
|---|---|---|---|---|---|---|---|
| | Coverage (g/m², on solids basis) | Coverage (g/m², on solids basis) | Metal salt | Amount mixed (parts) | Color reproduction | Ink absorption | |
| 1 | 10 | 5 | MgSO₄ | 8 | ⊚ | ○ | |
| 2 | 10 | 5 | MgSO₄ | 4 | ⊚ | ○ | |
| 3 | 10 | 5 | MgSO₄ | 2 | ⊚ | ○ | |
| 4 | 10 | 5 | MgSO₄ | 0.5 | ○ | ○ | |
| 5 | 10 | 5 | Al₂ (SO₄)₃ | 4 | ⊚ | ○ | |
| 6 | 10 | 5 | Na₂S₂O₃ | 4 | ○ | ○ | |
| 7 | 10 | 5 | Na₂SO₄ | 4 | ○ | ○ | |
| 8 | 10 | 5 | K₂S₂O₃ | 4 | ○ | ○ | |
| 9 | 10 | 5 | K₂SO₄ | 4 | ○ | ○ | |
| 10 | 10 | 5 | ZnSO₄ | 4 | ○ | ○ | |
| 11 | 10 | 5 | MgS₂O₃ | 4 | ○ | ○ | |
| 12 | 0.5 | 3 | MgSO₄ | 4 | ○ | Δ | |
| 13 | 30 | 5 | MgSO₄ | 4 | ⊚ | ⊚ | |
| 14 | 30 | 5 | MgSO₄ | 4 | ○ | ○ | Laminated paper was used as a support |

**Table 2**

| Comparative Example No. | First Layer | | | Second Layer (uppermost layer) | | | Evaluation Results | | |
|---|---|---|---|---|---|---|---|---|---|
| | Coverage (g/m2, on solids basis) | Metal salt | Amount mixed (parts) | Coverage (g/m2, on solids basis) | Metal salt | Amount mixed (parts) | Color reproduction | Ink absorption | note |
| not water soluble → 1 | 10 | - | - | 5 | MgCO₃ | 4 | × | ○ | |
| 2 | 10 | - | - | 5 | - | - | × | ○ | |
| 3 | 10 | MgSO₄ | 4 | 5 | - | - | × | ○ | |
| 4 | 10 | - | - | 5 | FeSO₄ | 4 | × | ○ | Ink receiving layer was colored |

### Dye Tnk Jet Recording Test

Solid black patterns were recorded on each of the recording materials prepared in Examples 1 and 5 by means of an ink-jet printer using dye ink, Model PM-770C (trade name, a product of Seiko Epson Corp.). The recorded areas were examined for metallic gloss. The results obtained are shown in Table 3.

**Table 3**

| | Metal salt mixed in uppermost layer | Metallic gloss |
|---|---|---|
| Example 1 | MgSO₄ | absent |
| Example 5 | Al₂(SO₄)₃ | present |

As can be seen from the results shown in Tables 1 to 3, the recording materials according to embodiments of the invention were well suited for ink jet recording processes for pigment ink, and ensured both high ink absorption and satisfactory color reproduction in the images recorded thereon.

## Claims

1. An ink-jet recording material having on a support at least two ink-receiving layers comprising pigment and binder, which is suitable for an ink-jet process using pigment ink: **characterized in that** the material further contains in the uppermost layer of the ink-receiving layers at least one water-soluble acidic or neutral metal salt selected from the group consisting of aluminium salts, magnesium salts, sodium salts, potassium salts and zinc salts, wherein the water-soluble metal salt is contained in an amount of 0.5 to 10 parts by weight per 100 parts by weight of pigment in the uppermost ink-receiving layer, and the constituent anion of the metal salt is a sulphate or thiosulfate ion.

2. An ink-jet recording material as described in claim 1, wherein the water-soluble metal salt is magnesium sulphate, aluminium sulphate, sodium thiosulfate or potassium thiosulfate.

3. An ink-jet recording material as described in claim 2, wherein the water-soluble metal salt is magnesium sulphate.

4. An ink-jet recording material as described in claim 2, wherein the water-soluble metal salt is aluminium sulphate.

5. An ink-jet recording material as described in claim 2, wherein the water-soluble metal salt is sodium thiosulfate.

6. An ink-jet recording material as described in claim 2, wherein the water-soluble metal salt is potassium thiosulfate.

7. An ink-jet recording material as described in any preceding claim wherein the water-soluble metal salt is contained in an amount of 0.5 to 8.0 parts by weight per 100 parts by weight of pigment in the outermost receiving layer.

8. An ink-jet recording material as described in any preceding claim wherein the uppermost ink-receiving layer has a coverage of at least 3g/m².

## Patentansprüche

1. Tintenstrahlaufzeichnungsmaterial, das auf einen Träger wenigstens zwei Tinte aufnehmende Schichten enthaltend Pigment und Bindemittel aufweist, das für einen Tintenstrahlprozess unter Verwendung von Pigmenttinte geeignet ist, **dadurch gekennzeichnet, dass** das Material darüber hinaus in der obersten Schicht der Tintenaufnahmeschichten wenigstens ein wasserlösliches saures oder neutrales Metallsalz enthält, das aus der Gruppe bestehend aus Aluminiumsalzen, Magnesiumsalzen, Natriumsalzen, Kaliumsalzen und Zinksalzen ausgewählt ist, wobei das wasserlösliche Metallsalz in einer Menge von 0,5 bis 10 Gewichtsteilen pro 100 Gewichtsteilen an Pigment in der obersten Tintenaufnahmeschicht enthalten und das konstituierende Anion des Metallsalzes ein Sulfat- oder Thiosulfation ist.

2. Tintenstrahlaufzeichnungsmaterial nach Anspruch 1, bei dem das wasserlösliche Metallsalz Magnesiumsulfat, Aluminiumsulfat, Natriumthiosulfat oder Kaliumthiosulfat ist.

3. Tintenstrahlaufzeichnungsmaterial nach Anspruch 2, bei dem das wasserlösliche Metallsalz Magnesiumsulfat ist.

4. Tintenstrahlaufzeichnungsmaterial nach Anspruch 2, bei dem das wasserlösliche Metallsalz Aluminiumsulfat ist.

5. Tintenstrahlaufzeichnungsmaterial nach Anspruch 2, bei dem das wasserlösliche Metallsalz Natriumthiosulfat ist.

6. Tintenstrahlaufzeichnungsmaterial nach Anspruch 2, bei dem das wasserlösliche Metallsalz Kaliumthiosulfat ist.

7. Tintenstrahlaufzeichnungsmaterial nach irgendeinem vorhergehenden Anspruch, bei dem das wasserlösliche Metallsalz in einer Menge von 0,5 bis 8,0 Gewichtsteilen pro 100 Gewichtsteilen an Pigment in der äußersten Aufnahmeschicht enthalten sind.

8. Tintenstrahlaufzeichnungsmaterial nach irgendeinem vorhergehenden Anspruch, bei dem die oberste Tintenaufnahmeschicht einen Bedeckungsgrad von wenigstens 3 g/m² aufweist.

## Revendications

1. Matériau d'enregistrement à jet d'encre, comprenant, sur un support, au moins deux couches de réception d'encre comprenant du pigment et du liant, adapté pour un procédé à jet d'encre utilisant de l'encre à pigments ; **caractérisé en ce que** le matériau comprend en outre dans la couche la plus supérieure parmi les couches de réception d'encre au moins un sel métallique acide ou neutre soluble à l'eau choisi dans le groupe comprenant les sels d'aluminium, les sels de magnésium, les sels de potassium, et les sels de zinc, dans lequel le sel métallique soluble à l'eau est contenu dans une proportion de 0,5 à 10 parties en poids pour 100 parties en poids de pigment dans la couche de réception d'encre la plus supérieure, et l'anion constitutif du sel métallique est un ion sulfate ou thiosulfate.

2. Matériau d'enregistrement à jet d'encre selon la revendication 1, dans lequel le sel métallique soluble à l'eau est du sulfate de magnésium, du sulfate d'aluminium, du thiosulfate de sodium, ou du thiosulfate de potassium.

3. Matériau d'enregistrement à jet d'encre selon la revendication 2, dans lequel le sel métallique soluble à l'eau est du sulfate de magnésium.

4. Matériau d'enregistrement à jet d'encre selon la revendication 2, dans lequel le sel métallique soluble à l'eau est du sulfate d'aluminium.

5. Matériau d'enregistrement à jet d'encre selon la revendication 2, dans lequel le sel métallique soluble à l'eau est du thiosulfate de sodium.

6. Matériau d'enregistrement à jet d'encre selon la revendication 2, dans lequel le sel métallique soluble à l'eau est du thiosulfate de potassium.

7. Matériau d'enregistrement à jet d'encre selon l'une quelconque des revendications précédentes, dans lequel le sel métallique soluble à l'eau est contenu dans une proportion de 0,5 à 8,0 parties en poids pour 100 parties en poids de pigment dans la couche de réception la plus supérieure.

8. Matériau d'enregistrement à jet d'encre selon l'une quelconque des revendications précédentes, dans lequel la couche de réception d'encre la plus supérieure a un rendement en surface d'au moins 3g/m².
